

## UNITED STATES PATENT OFFICE.

WINTHROP STANLEY LAWRENCE, OF BROOKLYN, NEW YORK, ASSIGNOR TO KAUMAGRAPH COMPANY, OF NEW YORK, N. Y., A CORPORATION OF NEW YORK.

## METHOD OF DECORATING LEATHER AND IMPROVED DECORATED LEATHER.

No Drawing.

Application filed January 26, 1927. Serial No. 163,580.

My invention relates to a new and improved method of decorating leather, and to a new and improved decorated leather.

One of the objects of my invention is to provide a method whereby leather can be decorated in one or more colors by a direct lithographic process so as to produce a maximum number of color combinations at a minimum expense.

10 Another object of my invention is to provide a method of decorating leather by a printing process which will permit the use of a variety of color combinations and which will prevent the ink from smearing upon the 15 surface of the leather.

Another object of my invention is to provide a new and improved form of decorated leather made according to my improved method, it being understood, however that 20 the claims herein for the new and improved decorated leather are not limited to any particular process for making the same.

Other objects of my invention will be set forth in the following description which illustrates a preferred embodiment thereof, it being understood that the above general statement of the objects of my invention is intended to merely generally explain the same, and not to limit it in any manner.

30 Various methods for decorating leather have been known for a great many years, but these methods have all been relatively expensive and they did not permit the ready and cheap application of designs in a great 35 many color combinations.

It has been proposed, for example, to apply a decorated design to leather by means of a dyeing process, but this method has been very expensive.

40 It has also been proposed to coat leather so as to provide a surface layer which will readily take up ink, but this method has proved impractical for decorating leather for various purposes, as for example, in making

45 "turn" shoes because the surface film did not stretch as readily as the moist leather, so that the surface film tended to crack and peel off when the leather was stretched.

According to my invention a great variety 50 of designs in a great many colors can be simply and efficiently produced by a direct lithographic or other printing process.

My invention is particularly applicable to 55 decorating thin skins such as calf skins and kid skins which are afterwards used for mak-

ing turn shoes, in making which it is necessary to moisten the leather so that it can be readily stretched.

According to my invention the individual skins are caused to adhere to bases made of thin bendable card board or paper by means of a binder or adhesive which is preferably insoluble in water. For this purpose a No. 3 and a No. 8 lithographic varnish, mixed with a suitable cobalt dryer can be utilized. The skins can be connected to these paper mounts or bases by means of the adhesive and then piled up and subjected to pressure until the adhesive has set at ordinary atmospheric temperature.

This lithographic varnish mixed with the dryer is a base for lithographic inks and it can be directly handled upon a lithographic press. Hence, the adhesive can be applied to the paper base by means of an ordinary lithographic press which is a decided advantage because the use of a lithographic press makes it possible to apply the adhesive to the paper base either continuously or in separated spots or lines.

Each skin is, therefore, caused to adhere to its paper mount or base in a perfectly flat condition. Since the edges of the skins often have a rounded contour because they have been taken from a portion of the body of the animal having a rounded contour, it is preferable to make V-shaped cuts in the edges of the skins whenever this is necessary, so as to cause each skin to lie perfectly flat and tightly adhere to its mount.

It is preferable to use an adhesive which is insoluble in water because some of this adhesive often creeps to the outer surface of the skin. If the decorating process is applied to leather which has a water soluble surface film, then this film flakes off when the leather is moistened in the process of turning a shoe or the like, and this injures the quality of the decoration.

Each combined mount and skin can now be fed to a lithographic press in the ordinary manner, or be printed by any other type of printing device.

However, in order to render decoration on the leather by a direct printing process (lithographic or otherwise) practical it is necessary to first subject many kinds of leather to a degreasing process even before the skin is connected to its mount, and it is also necessary to use certain special inks. This degreasing

60

65

70

75

80

85

90

95

100

105

110

process is not necessary with certain kinds of leather, such as mocha, lambskin and other leathers commonly designated as "suede".

I have discovered that unless kid and calf leathers are degreased by a suitable commercial process before they are printed upon, that the greasy substances present in a tanned calf skin or kid skin form a surface layer which penetrates the lithographic ink so as to prevent it from properly oxidizing and setting so that the decoration tends to smudge which, of course, would render the entire process impractical.

Even if such skins are subjected to the ordinary degreasing process before they are lithographed, a certain amount of grease always remains in the skin.

I have discovered that if ordinary printing or lithographic inks are employed in this process, that the grease present in such skins penetrates the marking or decoration, or affects the oxidizing of the printing or lithographic ink in some manner, so that the setting of the ink is very much retarded. This disadvantage is cumulative because it takes a certain amount of time for the greasy substances in the skin to penetrate or act upon the lithographic ink. Hence, if the printing or lithographic ink is caused to set very quickly it will be unaffected by the greasy residues in the skin, at least to such an extent that a permanent and non-spreading mark can be secured. On the other hand, unless the ink is caused to set quickly it is gradually affected by the greasy residues in the skin, so that the time of oxidizing or setting is very much increased and the final marking readily smudges.

Hence, the printing or lithographic ink should have a sufficient percentage of cobalt or other dryer added thereto so as to cause it to oxidize or set within twenty-four (24) hours. This figure is merely approximate and is merely given by way of example because such inks are not absolutely uniform even though they may be made according to the same formula.

I can, therefore, merely generally state that the ink should have a sufficient amount of dryer incorporated therein so that it should set before it is so softened or acted upon by the greasy residues in the skin as to make it impossible to secure a permanent marking.

Instead of using inks having the ordinary linseed oil base, it is preferable to use inks having a China wood oil base as these dry more quickly and give results much superior than when an ink having a linseed oil base is utilized. However, I do not wish to exclude from my invention the use of a linseed oil ink.

However, in using China wood oil inks, care must be taken not to utilize those pigments which have a chemical action upon the

China wood oil and cause it to thicken to such an extent that it cannot be utilized in the lithographic process. For example, highly acid pigments cannot be utilized in connection with China wood oil.

Experience has also shown that superior results are secured by choosing pigments which are ground much more finely than has been hitherto customary in making lithographic inks.

It was heretofore considered that carbon black could not be utilized as a pigment in printing upon leather, by a lithographic process or otherwise, because an ink embodying carbon black spreads or smudges quite readily when used for printing upon ordinary paper. It was, likewise heretofore considered that the lithographic process in particular could not be successfully used in printing upon a substance such as leather unless the leather were first provided with a smooth and impervious surface coating such as a lacquer or the like, because the paper which has been heretofore used in lithographic printing has had the pores thereof filled as much as possible by means of suitable fillers, sizing, and the like.

I have found, however, that a black lithographic ink in which carbon black has been incorporated can be utilized for printing directly upon leather, even though the leather has not been provided with an impervious surface film. The very fine carbon black particles which ordinarily each have an oily coating and also have a film of adsorbed air, cling to or unite very firmly with the degreased leather so as to provide a very clear and permanent marking, so that the action of the leather is wholly different from that of ordinary paper in this respect.

In order to cause other pigments to unite with or adhere to the leather so as to afford a secure and permanent marking, it is necessary to grind such other pigments to a much greater degree of fineness than has hitherto been practiced, before incorporating the pigment in its oily vehicle. For example, other pigments should be ground until about 75% of the particles are smaller in size than four (4)  $\mu$ , namely, .004 mm. I believe that these very fine particles of pigment are adsorbed to a certain extent by the leather so as to afford a very clear and permanent marking while coarser particles are not sufficiently adsorbed by the leather so that they form a marking which can be easily blurred or smudged. Examination has shown that in printing with an ink containing carbon black, or containing pigments which has been ground to sufficient fineness, that the carbon black or other pigment penetrates the surface of the leather to form a durable marking. I include letter-press and other printing methods in my invention. That is, the ink is absorbed to a certain extent by being applied directly to

the porous surface of the leather and by making the pigment particles substantially fine they are carried along with the ink below the surface of the leather to a certain extent.

5 If any of the particles of pigment remain upon or above the surface of the leather they are so fine that the decorative marking produced does not smear.

After the greaseless or partially degreased 10 leather has been decorated according to my process by applying directly to the surface thereof an ink having the characteristics before mentioned, the decorated surface of the leather is finished in any suitable manner such as by giving it a lacquer coating or 15 the like.

It is not necessary that the leather should be connected to a mount before printing thereon but this is preferable as the leather 20 is much more easily manipulated. However, when the leather is connected to a mount the adhesive should be properly chosen so that it should not enter the pores of the leather and stiffen it. If, for example, the 25 leather becomes impregnated with an adhesive consisting of a drying oil such as linseed oil, then this oil becomes gradually oxidized so that the sheet of leather is stiffened. Likewise, although satisfactory results can be 30 secured if the leather is connected to the mount by a water soluble adhesive, this adhesive must be of a character which will not enter the pores of the leather to stiffen it. By using a suitable lithographic varnish having 35 a sufficient amount of dryer therein, the varnish previously mentioned can be caused to set without entering the pores of the leather so as to leave greasy spots thereon and stiffening the leather. If a water soluble adhesive

such as starch is employed this must be used 40 very sparingly so that it will not enter the pores of the leather to stiffen it.

I have described a preferred embodiment 45 of my invention, but it is clear that numerous changes and omissions could be made without departing from its spirit.

I claim:—

1. A method of decorating an unfinished 50 and commercially degreased leather which consists in connecting the leather to a mount by means of an adhesive non-soluble in water and then applying an ink having an oily base and a pigment directly to the exposed surface of the leather and before it is separated from its mount.

2. A method of decorating an unfinished 55 and commercially degreased leather which consists in connecting the leather to a mount by means of an adhesive, causing the adhesive to set without permitting it to enter the pores of the leather to an extent sufficient to substantially stiffen the leather, and then applying an ink having an oily base and a pigment directly to the exposed surface of the leather and before it is separated from its mount.

3. A method of decorating unfinished 60 leather which consists in connecting the leather to a mount by means of an adhesive embodying a drying oil, causing the adhesive 70 to set without permitting it to enter the pores of the leather to an extent sufficient to substantially stiffen the leather and then printing on the exposed surface of the leather before it is separated from its mount.

In testimony whereof I affix my signature.

WINTHROP STANLEY LAWRENCE.